

June 2, 1936.

W. L. STAFFORD  
THERMAL INSULATING STRUCTURE

2,042,870

Filed May 27, 1932

Fig. 1.



Fig. 2.



Fig. 3.



Fig. 4.



Fig. 5.



INVENTOR  
William L. Stafford.  
BY  
D. N. Halstead  
ATTORNEY

## UNITED STATES PATENT OFFICE

2,042,870

## THERMAL INSULATING STRUCTURE

William L. Stafford, Somerville, N. J., assignor to  
 Johns-Manville Corporation, New York, N. Y.,  
 a corporation of New York

Application May 27, 1932, Serial No. 614,133

4 Claims. (Cl. 72—35)

This invention relates to a monolithic thermal insulating structure and method of making the same, and particularly to such a structure comprising a casting of an insulating concrete integrally united at one face of the casting to a heat-resistant facing material.

An object of the invention is to make a monolithic thermal insulating wall that may be used in a furnace without an independent protecting layer interposed between the insulating wall and the source of heat. A further object is to provide a monolithic, rigid, and relatively impermeable insulating layer and a monolithic layer of facing material adapted to withstand higher temperatures than the insulating layer, the two layers being integrally united and adherent to each other over a wide range of temperature. An additional object is to provide a method of combining the insulating with the more refractory material in such manner as to produce a zone of graded mixing whereby abruptness of change in properties between the two layers is minimized.

There is a decided preference in thermal insulation for cellular material containing small pores or voids. An example of such insulation is diatomaceous earth, in which the pores are of microscopic size. An objection to such insulation is that it is not sufficiently refractory for all purposes, as for direct exposure to very high furnace temperatures. For this reason it is customary to protect diatomaceous earth insulating material with a layer of firebrick or other refractory material interposed between the diatomaceous earth product and the source of heat, or to use the diatomaceous earth insulation at temperatures not above those which can be withstood by the product without protection.

To protect cellular insulating products from the slagging action of furnace gases or from abrasion, there has been used heretofore a firebrick wall, as stated, or, if the temperature is not excessive, a wash of a cementitious product. The cementitious coating has been used in the form of a thin layer that does not show much temperature difference between the outside of the coating and the back side which adjoins the insulating material.

There has also been described a refractory insulating material containing pores, such as those produced by heating an earthy product containing a substance adapted to develop gas, with the consequent formation of pores or voids, on heating. Such a refractory insulating material containing relatively large voids has been used in combination with similar and equally refrac-

tory but impervious facing, in order to prevent the entrance of material into the voids, as, for example, from a furnace which is insulated with the material containing the voids.

An example of a thermal insulating product containing small pores is that made as described in U. S. Patent 1,184,184 to Krieger. This product consists of fragments of kieselguhr (diatomaceous earth) in a partially fritted condition and a binder. A preferable form of such insulation is made by first calcining diatomaceous earth in lump form at approximately 1900 to 2000° F., cooling, and granulating and screening to 3 mesh and finer, suitably with a small proportion only or none of the material finer than 50 mesh. Four volumes of this granular calcined diatomaceous earth are then mixed with about 1 volume of Portland cement and sufficient water to give a workable concrete. The proportion of water may be varied to give the consistency desired. For many purposes the water used in the mixture may be approximately 60 to 70% of the dry weight of the solids in the concrete. When this wet concrete is cast and allowed to stand until the hydraulic cementitious material becomes hard, there results an insulating diatomaceous concrete having a specific thermal conductance of about 2.4 British thermal units at a mean temperature of 1000° F. When the hardened product is used in a furnace wall, it is found that the concrete is non-refractory and that disintegration by heat becomes important when the outside of the hot surface, that is, the surface directed towards the source of heat comes to have a temperature of about 1700 to 1900° F.

From the following description of the present invention it will be seen that there has now been constructed a monolithic thermal insulating wall comprising a diatomaceous earth concrete that may be used at a hot surface temperature that is very substantially higher than that at which the usual insulating concrete construction is satisfactory.

A preferred embodiment of the invention is illustrated in the drawings in which

Fig. 1 is a side elevational view of a monolithic insulating structure adapted for use as a wall, such as a floor of a furnace.

Fig. 2 is an end elevational view of a granular calcined diatomaceous earth and Portland cement concrete casting with irregularities on one face adapted to increase the firmness of union of a later to be applied heat-resistant facing.

Fig. 3 shows an end elevational view of a thermal insulating and heat resisting structure

adapted for use as a side wall of a furnace and consisting of the insulating layer shown in Fig. 2, with the heat-resistant facing applied to one face thereof in such manner as to fill the irregularities 5 of the surface of the insulating layer.

Fig. 4 is a view of a furnace, partly diagrammatic and broken away, for clearness of illustration. The firebox in this furnace is insulated at the front (left) side and the bottom with the 10 structure of the present invention.

Fig. 5 shows an enlarged end elevational view of a portion of the structure illustrated in Fig. 1, and particularly an intermediate zone of graded mixing.

15 In the various figures, like reference characters refer to like parts. Thus the thermal insulating structure comprises Portland cement 1, granules of calcined diatomaceous earth 2, a heat-resistant layer 3 united integrally to a face 20 of the calcined diatomaceous earth and Portland cement concrete, and extensions into or mixtures 4 of the heat-resistant material with the said concrete in an intermediate zone between the heat insulating material on one side and the 25 more refractory material on the other. When the thermal insulating material is to be used in a side wall and when it must be cast in an upright position, the casting of the insulating material may be made, allowed to take its initial set, and then provided with irregularities of surface such as those shown at 5 in Fig. 2, into which the heat-resistant material may be forced during the application of the latter to the insulating wall. When these irregularities are filled with the 30 facing material, there are formed extensions 6 of one material into the other. When the sides of the irregularities are of such slope as to produce an opening which is more narrow than the back part or the base of the irregularity, there is 35 produced a dove-tailing effect, illustrated in Figs. 3 and 4, which favors the firm anchorage of the heat resistant facing to a face of an upright layer of insulating material.

The application of the structure of the present invention to a furnace, such as a domestic oil-fired furnace, is illustrated in Fig. 4. It will be seen that the combustion chamber 8 is insulated at the front or left side with insulating concrete containing granular calcined diatomaceous earth and Portland cement, the concrete being protected from direct radiation from the combustion chamber by means of an integrally 50 united heat-resistant layer coated over and into the irregularities of surface of the insulating wall. The bottom of the furnace is insulated 55 with a structure of the type illustrated in Fig. 1. The back side of the firebox, against which the flame from fuel entering through the pipe 7 may strike directly, is constructed in conventional manner, with the insulating concrete protected by a wall of firebrick 9.

Fig. 5 illustrates a detail which is not so evident in the other figures, all of which are drawn to a smaller scale. In Fig. 5 it will be seen that 60 there may be an intermediate zone 10 of graded mixing between the insulating layer on the one side and the heat-resistant or more refractory layer on the other side.

70 The invention is illustrated by the following examples.

#### Example 1

A monolithic thermal insulating structure, suitable for use in the door of a furnace, is constructed as follows.

5 Into a mold, or form of interior size and shape desired for the insulating structure, there is cast a wet (water-containing) concrete comprising 4 parts by volume of granular calcined diatomaceous earth (so-called "C-3") to 1 part by 10 volume of Portland cement. This concrete is cast to a depth that may be varied with the thoroughness of insulation desired. A depth that is satisfactory for most purposes is 5 inches. On top of this casting, and before the casting 15 has hardened, there is poured a wet mixture containing, besides water, approximately 75 parts by weight of fireclay grog, 2 parts of diaspore, and 23 parts of a quick hardening, high alumina hydraulic cement (so-called "Lumnite" 20 cement, cement fondu, or calcium aluminate cement). The thickness of this layer of materials may be approximately a third of that of the insulating layer, say  $\frac{1}{2}$  to 2 inches, suitably about 1 to  $1\frac{1}{2}$  inches. This material, while not a true 25 refractory or adapted to withstand high furnace temperatures, is more heat-resistant than the insulating concrete and is adapted to withstand temperatures up to about 2300 to 2500° F.

For best results, the Portland cement and 30 granular calcined diatomaceous earth concrete is made up with a proportion of water that gives a fairly thick mixture, whereas the heat-resistant material of the kind described is made up with water to a fairly thin slurry.

35 After the water mixtures of both the insulating and the more refractory materials have been poured, the upper layer of heat-resistant material is pushed down at intervals into the floor layer, as by repeatedly inserting and withdrawing a rod endwise, at intervals. This is sometimes referred to as "rodding". This rodding, or pushing down, produces extensions of the refractory material into the insulating layer, as illustrated at 4 in Fig. 1, and also gives some 40 mixing, to form an intermediate zone of graded mixing, approximately as illustrated at 10 in Fig. 5.

45 After this rodding is completed, the mixture is allowed to stand at atmospheric temperature, that is, without the application of external heat, until the two layers have hardened. It should be added that the Lumnite cement, and also the Portland cement to a lesser extent, are warmed somewhat by the heat developed during the setting. After hydraulic hardening, heat may be applied.

50 The structure so made may be installed in the metal shell of a furnace door.

#### Example 2

55 The procedure and materials are the same as under Example 1, with the exception that the heat-resistant material is first added to form a layer that is relatively thin, as, for example,  $\frac{1}{2}$  inch. This thin layer is then partly stirred into the top portion of the lower layer containing the insulating concrete, to give a mixed layer, after which there is then added the rest of the heat-resistant material, to give a total thickness 60 of layer of such material about equal to that produced in Example 1.

#### Example 3

65 Forms are erected and a conventional mixture 70 of granular calcined diatomaceous earth and Portland cement is cast in edgewise position to produce a slab suitable for use as a side wall. (It will be understood that it is frequently necessary to cast these walls directly in the position 75

in which they are to be used, and for this reason it is not feasible in all cases to cast the wall in the position shown in Fig. 1 and then elevate it into place in the side of a furnace.) After the 5 side wall casting has set, it may be notched roughly, as shown at 4 in Fig. 2, to provide irregularities adapted to facilitate the later bonding of a heat-resistant facing thereto. For convenience, these notches may be shaped roughly during the casting 10 operation by having blocks of wood project into the form at selected locations. After the casting is set and the forms with the attached blocks of wood are removed, the irregularities may be shaped with a chisel, to produce side 15 walls that converge in the direction of the face of the block provided with the irregularities or depressions. After the irregularities have been formed, or directly after the casting has partially hardened, in case no irregularities are to be used, 20 there is applied to the face of the wall, which during use is to be nearest to the source of heat, a layer of refractory or heat-resistant material of the kind described under Example 1. In applying this layer of heat-resistant material to one face 25 of the insulating concrete, one side of the form which was used originally for retaining the Portland cement and granular calcined diatomaceous earth concrete may be moved back, that is, away from the face, a sufficient distance to allow casting 30 a layer of heat-resistant material of the desired thickness between the face of the concrete and the form in its new position. Or the heat-resistant layer may be applied in some cases by trowelling on. However, the latter method is 35 somewhat complicated by the fluidity of the mixture of the heat-resistant material and water at the time the heat-resistant material is applied. This difficulty may be minimized by trowelling on 40 and allowing the heat-resistant material to take its initial set in several successive thin layers instead of one thick layer.

The properties of the insulating structure made according to the present invention are such as to adapt it to extensive commercial use as a means 45 of restricting the flow of heat. Thus the insulating layer of the structure has its usual efficiency as a thermal insulator. Also, the heat-resistant layer is sufficiently thick to offer substantial resistance to the flow of heat. While this may not be so very important directly in the total resistance 50 of the structure to heat transfer, it is important in lowering substantially the temperature on the hot side of the layer of insulating material. With this structure there is produced a wall that 55 will withstand 300 to 600 degrees F. higher temperature on the hot surface than is the case when the heat-resistant layer is omitted and the conventional, thermal insulating, granular calcined diatomaceous earth concrete is used without a protecting layer. It will be understood that the extent 60 of the increase in temperature that may be withstood by the wall will vary in part with the thickness of the heat-resistant layer. In general, when increased temperature resistance is desired, there should be avoided very thin wash coatings, such as have been used heretofore, over insulating 65 brick walls, for other purposes than that of increasing the resistance to high temperatures.

The insulating material in the present structure 70 contains a cellular or void-containing product, such as the granular calcined diatomaceous earth, which is bonded together by non-refractory cementitious material hardened by setting at at-

mospheric temperature. The wall has satisfactory resistance to crushing.

The insulating layer itself is rigid and has substantial strength and resistance to crushing. 5 Also, it may be relatively impermeable, that is, it is not readily permeated throughout by water; pores or porous material in the insulating layer are enclosed by cement, in the preferred embodiment of the invention, to give an overall effect of non-porosity. The cellular particles may be embedded in and surrounded by non-porous material. 10

Maintaining the integral union, over a wide range of temperatures, of a rigid facing layer and an insulating layer that is also rigid, involves a 15 problem that is absent when the insulating layer is more or less yieldable and adapted to undergo change of shape or volume under the influence of stresses of even minor magnitude and without cracking. The problem is further complicated 20 when the insulating layer contains a high proportion of Portland cement. A Portland cement casting, when heated through a wide temperature range, shows an unusual volume change. Thus, 25 there is contraction during one stage, possibly while the cement is losing water, followed by expansion at higher temperatures.

In spite of these difficulties, the present invention provides a structure, comprising a rigid insulating concrete integrally united to a rigid facing of different material, that does not crack apart or separate as the temperature of the structure is varied, for example, from atmospheric up to furnace temperature. Thus, a furnace containing 30 such a structure may be heated or cooled, say, 35 from 2300 to 2400° F. on the hot face to atmospheric temperature, without destroying the bond between the layers of the two different materials.

The heat-resistant material, comprising a high proportion of the granular fireclay grog and a 40 lesser proportion of the cementitious material of the quality of Lumnite, not only hardens when its wet mixture is allowed to stand, but also probably undergoes partial fritting or vitrification of its 45 outside surface on being strongly heated. The final set of the outside surface of the heat-resistant material is partly ceramic in nature and is not developed fully until after the wall structure including the Portland cement has been heated. 50

In a modification of the invention, the casting, with its heat-resistant facing and insulating backing containing hydraulic cementitious material may be subjected to an elevated temperature before the cementitious material has taken its 55 final set.

In place of the granular calcined diatomaceous earth there may be used some other insulating material, suitably one containing voids or cells and made into granular form. Thus, there may 60 be used the product described in U. S. Patent 1,812,376 to Ross and Lambie, and comprising a porous refractory material produced by heating cyanite. Or there may be used, in place of the diatomaceous earth, a product made, as described 65 in U. S. Patent 1,583,521 to Boynton, by heating a slurry of earthy material that develops gas during such heating. In cases where the insulating layer is not to be exposed to high temperatures, granular diatomaceous earth that has not been 70 calcined may be used.

In place of the Portland cement in the insulating concrete, there may be used another binding material. Thus, there may be used the calcium aluminate cement described above, although 75

the use of the latter is at present not recommended because of its cost.

In place of the insulating concrete containing granular calcined diatomaceous earth, there may be used a concrete containing voids, such as a concrete sold under the name "Porete" and made by casting a mixture of cement, water, a foam producing and stabilizing substance, and air, the air being in the form of bubbles or foam distributed throughout the rest of the material. Such voids, however, are not as effective in heat insulation at high temperatures as the smaller pores in diatomaceous earth. Such a concrete containing voids should not be used in structures in which the concrete is exposed to temperatures at which Portland cement fails.

It is preferred to use an insulating and also heat-resisting layer containing each a large proportion of granular material and a lesser proportion by volume of binding agent. The explanation for the better adherence obtained with the high proportion of granular material (granules in the insulating layer and grog in the heat-resistant layer) and the minimized tendency to separation with change of temperature may be the effect of the granules in localizing the tendency to cracking of the structure with changes in temperature and/or in making the layer containing the granules somewhat less brittle.

In place of the Lumnite cement, in its mixture with diaspore and fire-clay grog, as the facing material, there may be used another cementitious material, as, for example, a double calcined, high lime content cement, suitably containing 65 to 69% of lime, calculated as calcium oxide, and sold under the name "Incor" cement. Incor cement and grog compositions are less refractory than Lumnite cement and grog compositions.

As a substitute for the diaspore there may be used another hydrous mineral aluminum oxide or hydroxide, as, for example, ground raw bauxite. The diaspore, or aluminum oxide or hydroxide, serves the function of increasing the workability of the mixture that is cast. If this function is not desired or necessary, such materials may be omitted from the composition.

The fireclay grog which has been described as being used as a major ingredient of the heat-resistant mixture is a refractory and is suitably 6-mesh and finer but free from any large proportion of very fine material. As grog, there may be used a refractory aggregate having a suitably low coefficient of thermal expansion, as, for ex-

ample, fused alumina, mullite, silicon carbide, as substitutes for the fireclay grog, in whole or in part.

Since many variations from the illustrative details given may be made, it is intended that variations within the spirit of the invention should be included within the scope of the claims.

What I claim is:

1. A monolithic thermal insulating structure comprising a thermal insulating layer, containing a cellular material and Portland cement hardened by setting at approximately atmospheric temperature, and a heat-resistant facing layer integrally united to the insulating layer, said facing layer containing a large proportion of granular refractory material and a lesser proportion of a hydraulic cementitious material.

2. A thermal insulating structure comprising in combination a monolithic casting of a mixture of granulated calcined diatomaceous earth and Portland cement and a heat-resistant protective layer of facing material containing approximately 75 percent of calcined fireclay grog, approximately 2 percent of a hydrous aluminum oxide, and approximately 23 percent by weight of calcium aluminate cement.

3. A thermal insulating, heat-resisting structure comprising in combination a mixture of lightweight granules and a binder therefor, of the type of hardened Portland cement, a protective facing material adapted to withstand higher temperatures than the said mixture and adhered thereto, and an intermediate zone of graded mixing between the mixture and facing material, whereby there are eliminated marked inequalities of coefficient of thermal expansion between adjacent portions of the structure.

4. A monolithic thermal insulating structure comprising a thermal insulating layer, containing granular calcined diatomaceous earth of particle size finer than approximately 3-mesh and Portland cement in the proportion of approximately one volume of the cement to four volumes of the calcined diatomaceous earth, and a heat-resistant facing layer integrally united to the insulating layer, said facing layer containing a large proportion of granulated calcined fireclay and a lesser proportion of a hydraulic cement of high alumina content and being adapted to adhere to the said insulating layer over a wide range of temperatures extending from atmospheric to about 2300° F.

WILLIAM L. STAFFORD.